

## UNITED STATES PATENT OFFICE.

THEODORE F. BRADLEY, OF CRANFORD, NEW JERSEY.

## PROCESS OF DE-LIVERING PAINTS, VARNISHES, AND THE LIKE.

No Drawing.

Application filed August 23, 1921. Serial No. 494,687.

*To all whom it may concern:*

Be it known that I, THEODORE F. BRADLEY, a citizen of the United States, residing in the city of Cranford, county of Union, State 6 of New Jersey, have invented certain new and useful Improvements in Process of De-livering Paints, Varnishes, and the like, of which the following is a specification.

This invention relates to what is technically referred to in the paint and varnish industry as de-livering, and involves the treatment of varnishes or paints having varnish wholly or partly as a vehicle, in order to maintain the desired viscosity, or in the 10 case of paint or varnish that has thickened partly to bring it back to a good working consistency. This I accomplish by treating with material which accomplishes the very much desired object, but without any undesirable or deleterious effects.

It is well known that paints and varnishes in very large quantity often thicken and become largely a waste or loss, and to prevent their reaching this condition, or if 15 in a partially livered state, to bring them back to good working consistency is of great value, and attempts heretofore to accomplish the result have been either only partial or with attending objectionable effects.

One particular embodiment of my invention I will now describe, which consists in adding free fatty acids such as are obtained, for instance, from vegetable oils, to a varnish or a paint whose vehicle consists either wholly or partly of varnish. In the case of 20 a paint, I add from half of one per cent to ten per cent by weight of linseed oil fatty acids, having a specific gravity, for example, of .9200 at 15° centigrade and having an acid value of 170. The exact proportion needed depends upon the condition and composition of the paint at the time it is treated. In the case of a varnish, a smaller 25 proportion, seldom more than eight per cent, has the desired effect, and the de-liverer is particularly effective on varnishes of the China wood, that is the tung oil type, and especially in the case of those having a so-called "false body." The free fatty acid 30 may be added either as such or in the form of an acid oil containing the necessary amount of free fatty acid.

The addition of fatty acids as obtained 35 from vegetable oils I find is particularly

effective in the case of those obtained from linseed or tung oils. While other acids, such as rosin acids will act similarly, the best results are obtained with fatty acids.

This de-liverer or thinner is non-volatile, 40 and can therefore be classed among fixed oils. By the addition of this relatively small proportion by weight, my process of de-livering is accomplished without very material increase in volume of paints, varnishes or the like, and, in fact, so little fatty acid is required in my process to accomplish 45 the desired purpose, that there is no great reduction in opacity, which objectionable characteristic would be caused in the case 50 of adding turpentine or similar volatile thinner.

In the case of over-cooked varnishes, this process is particularly efficacious because they can be brought back to a proper viscosity of the varnish without the objectionable addition of large relative amounts of volatile thinner, which makes my process especially valuable in the manufacture of 55 tung oil varnishes.

Paints and varnishes treated with fatty acids of vegetable oils are not greatly altered in composition, which otherwise would be the case were relatively much volatile thinner used. Heretofore, this has 60 been the only process of accomplishing any satisfactory thinning effect.

Heretofore it has been thought that the thickening of paint is due to reaction between free acid of the vehicle and the basic 65 matter of the pigment, forming insoluble salts which were the cause of the thickening.

I find, however, that in vehicles which consist wholly or partly of a varnish where chemical reaction takes place and thickening occurs, it is due but little to the presence of insoluble salts, but is mainly due to a decrease in the dispersion of the varnish. This dispersion of the varnish in turn is reduced by the partial or complete neutralization 70 of the free acid of the vehicle by basic material in the pigment. The complete neutralization does not occur in any except a very few cases, due to the presence of protecting colloids, (the gums and oils). When fatty or rosin acids are added to such a paint the vehicle regains its original degree of dispersion, and it thereafter reacts but little due to the presence of the protecting colloids. Consequently paints of a highly 75

basic nature may be successfully treated by my process.

The solution of the problem accomplished by my process, it will thus be seen, results from my determination that the acid value, namely, the relative amount of free acid present in a varnish, is one of the factors determining the viscosity. In view of this the reasons are better understood for differences in paint consistencies and varnish viscosities.

This will be further understood when we consider that the viscosity, or, as frequently referred to, the body of the varnish is dependent upon the number of particles of gum per unit volume, the relative size of the gum particles, the state of polymerization of the oils and the amount of free acid present. Thus if turpentine or similar thinner be added the volume of the liquid is materially increased with an attendant decrease in the number of gum particles per unit volume; whereas with the addition of fatty acids the gum particles are decreased in size, polymerized oils are properly dispersed and decreased in mass,—so that the thinning effect is accomplished by my process although the original volume of the liquid is but slightly increased.

30 The drying time and the finish and durability of the varnish or paints are not materially affected, so that neither these nor reduction in opacity, nor any other deleterious effects result from the practice of my invention. The pigments involved in paints are likewise not affected, so that the net result of my invention affords a highly advantageous process in the treatment of substantially all paints containing varnish and varnishes in order to either maintain their proper consistency or to bring them back to the proper consistency after overcooking, or after they have livered as a result of time or other outside effect.

45 The addition of a suitable relative amount of free fatty acids is made by pouring the required amount into the paint or varnish, and with suitable stirring the effect throughout the mass or volume gives quick results.

50 While the efficacy of my process will naturally vary somewhat with different paints and varnishes, a wholly satisfactory effect is obtained within reasonable limits as hereinbefore set forth, by appropriate variations in the relative quantity of fatty acids added for either paints or varnishes, and under a reasonable range of temperature and other conditions.

60 My process can also be applied to printers' inks, lithographers' inks, and similar inks, and my de-liverizing agent has been found very useful in thinning down these inks, and preserving them at, or bringing them to any desired consistency.

65 Without limiting myself to the specific

practice of my invention heretofore set forth, what I claim and desire to secure by Letters Patent is:

1. A process for de-delivering coating materials containing a varnish vehicle, consisting in the addition of an amount of fatty acids substantially not exceeding ten per cent of the livered quantity of said coating material.

2. A process of preventing the livering of coating materials containing a varnish vehicle, consisting in the addition of not over substantially ten per cent by weight of a free fatty acid.

3. A process for preserving the consistency of coating materials containing a varnish vehicle, or restoring their consistency when partially or wholly livered, consisting in the addition of the fatty acid from linseed oil.

4. A process for preventing the alteration in viscosity of varnish, consisting in the addition thereto of approximately eight per cent by weight of the fatty acid of a vegetable oil.

5. A process for preventing the alteration in viscosity of varnish consisting in the addition thereto of approximately eight per cent by weight of the fatty acid of linseed oil.

6. The process of chemically restoring heavy-bodied varnish to a thinner consistency, comprising the admixture thereto of an amount not greater than approximately eight per cent of the fatty acids from vegetable oils.

7. The process of chemically restoring heavy-bodied varnish to a thinner consistency, comprising the admixture thereto of an amount not greater than approximately eight per cent of the fatty acid from linseed oil.

8. The process of restoring heavy-bodied varnish to a thinner consistency, comprising the admixture thereto of an amount of non-volatile fixed oil of an acid nature whose free acid content is not greater than approximately ten per cent of the varnish.

9. A process for preventing the change in the consistency of varnish, consisting in the addition thereto of an amount of non-volatile fixed oil of an acid nature whose free acid content is not greater than approximately ten per cent of the varnish.

10. A process for preserving the consistency of coating materials containing a varnish vehicle, consisting in the addition thereto of an amount of non-volatile fixed oil of an acid nature whose free acid content is not greater than approximately ten per cent of said coating material.

11. The process of restoring livered coating materials containing a varnish vehicle to previous relatively thin condition, consisting in the mixing therewith of an amount

of non-volatile fixed oil of an acid nature whose free acid content is not greater than approximately ten per cent of said coating material.

6 12. A process for preserving the consistency of coating materials containing a varnish vehicle or restoring their consistency when partially or wholly livered, which consists in the addition thereto of not over approximately ten per cent by weight of the fatty acid of a vegetable oil.

10 13. A varnish containing the usual ingredients and approximately eight per cent of fatty acids of vegetable oils.

14. A varnish containing the usual ingredients and between one and eight per cent of fatty acids of vegetable oils.

15. A varnish containing the usual ingredients and approximately eight per cent of fatty acids of linseed oil.

In testimony whereof, I have signed my name to this application, in the presence of two subscribing witnesses, this 20th day of August 1921.

THEODORE F. BRADLEY.

Witnesses:

J. H. CUNTZ,  
HERMAN F. CUNTZ.